# EUROPEAN PATENT SPECIFICATION

(11) **EP 1 863 959 B1**
(45) Date of publication and mention of the grant of the patent: **21.08.2019**
(21) Application number: 06726385.5
(22) Date of filing: 13.03.2006
(51) Int. Cl.: D04B 21/02

(54) **IMPROVEMENTS IN OR RELATING TO SPACER FABRICS**
VERBESSERUNGEN BEI ABSTANDSSTOFFEN
AMELIORATION APPORTEE OU RELATIVE A DES TISSUS D'ESPACEMENT

(30) Priority: 22.03.2005 GB 0505839
(43) Date of publication of application: 12.12.2007
(73) Proprietor: MOTHERCARE UK LIMITED, Watford Herts WD2 5SH (GB); Heathcoat Fabrics Limited, Devon EX16 5LL (GB); Relyon Limited, Cheltenham Gloucestershire GL50 3SH (GB)
(72) Inventor: KEITCH, George, Shoreditch TA3 7BN (GB)
(74) Representative: Barker Brettell LLP
(86) International application number: PCT/GB2006/000896
(87) International publication number: WO 2006/100434

(56) References cited:
- EP-A- 0 994 207
- WO-A-01/11127
- WO-A-01/11128
- DE-A1- 19 910 785
- US-A- 5 870 785
- US-A1- 2003 106 346

## Description

This invention relates to spacer fabrics and more particularly to a novel spacer fabric and a mattress cover and composite mattress construction produced therefrom.

Spacer fabrics have opposite face structures united and held in spaced disposition by linking spacing threads. Spacer fabrics are known, for example, from GB2042003, which describes a liquid absorbing textile product, WO95/16416 which describes a compression bandage, WO95/12018 which describes clothing articles, US5896758 which describes a fabric for footwear and backpacks, WO99/05990 which describes a prosthetic fabric, WO96/01602 which describes a mat, and US5834382 which describes a high temperature resistant covering. The entire disclosures of all these patents are incorporated herein by reference for all purposes.

In UK Patent No. GB2305191B there is described and claimed a flexible spacer material, which comprises a fabric, providing a liquid permeable and breathable upper surface and a heat and liquid dissipating spacer layer, and a liquid impermeable lower surface layer. The spacer material is used for the production of mattress covers and more particularly for cot mattresses for babies and young children.

In European Patent No. 1204791B there is described and claimed a flexible spacer fabric, the fabric having a liquid permeable and breathable upper surface layer, the upper surface layer comprising a knitted mesh wherein the average width of the mesh strands in the upper surface layer is from 0.1 mm to 4 mm and wherein the ratio of average hole diameter to average strand width is from 4:1 to 1:2, a heat and liquid dissipating spacer layer, and a dimensionally stable lower surface layer.

In UK Patent No.2352735B there is described and claimed a flexible spacer fabric, the fabric having a liquid permeable and breathable upper surface layer, the upper surface layer comprising wicking fibres and/or comprising a wicking fibre construction, a heat and liquid dissipating spacer layer, and a dimensionally stable lower surface layer.

Cot mattresses produced using the spacer materials and fabrics described in GB2305191B, EP1204791B and GB2352735B have vastly improved properties over conventional cot mattresses and the products, sold under the name SLEEPRIGHT (RTM) cot mattress by Mothercare UK Limited, have proved to be commercially extremely successful.

Aspects of cot mattresses for infants that are extremely important include breathability, which gives an improved safety factor for the cot mattress, and air flow, which reduces the risk of over-heating, thereby leading to greater comfort for the infant. Also important are the liquid transport properties of the fabric, which ideally should enable rapid conveyance of body fluids away from the body region, reducing discomfort for the infant.

A further factor that influences the acceptability of a cot mattress is the "feel" of the fabric surface, which should preferably be smooth and soft to the touch. In this respect an improvement in the handle and feel of the existing products would be desirable. The existing fabric has an upper surface layer comprising a knitted
mesh which does not sit flat to the surface and does not have a soft "woven fabric" handle and feel. Nevertheless, the properties of breathability, air flow and liquid transport are inextricably linked to surface design and it has hitherto been found very difficult to provide improved softness of feel and handle without prejudicing the other desirable properties of the cot mattress. Attempts to improve the soft feel of the upper surface layer by brushing, for example, have not proved to be successful.

The present invention provides a flexible spacer fabric having a smooth, relatively flat, upper surface comprising a knitted mesh that emulates the soft feel and handle of a woven fabric, whilst substantially maintaining, or enhancing, the above-mentioned other desirable properties.

In a first aspect, the present invention provides a flexible spacer fabric, the fabric having a liquid permeable and breathable upper surface layer, a heat and liquid dissipating spacer layer, and a dimensionally stable lower surface layer, wherein the upper surface layer comprises a knitted mesh comprising sinusoidal mesh strands extending in parallel across the upper face of the fabric, said strands being spaced apart and linked at adjacent points by one or more straight threads forming holes, bounded by the mesh strands and threads, of generally oval shape, wherein the average width of the mesh strands in the upper surface layer is from 0.1 mm to 4 mm, and the parallel sinusoidal strands are offset from one another lengthwise, such that a peak of one strand faces a trough or an adjacent strand, characterised in that facing peaks and troughs are joined by four or more threads, to form the oval-shaped holes.

In a further aspect, the invention provides a mattress cover which comprises a flexible spacer fabric according to the invention and a liquid impermeable lower surface layer.

In another aspect the invention provides a cot mattress comprising a foam plastics core or a spring mattress core and a cover comprising an outer layer of flexible spacer fabric according to the first aspect of the invention and a liquid impermeable inner layer.

Preferred fibres for use in the upper surface layer are multifilament synthetic yarns. Suitable synthetic fibres include polyesters and polyamides, although polyesters are preferred, due to their greater heat stability. Preferred multi-filament yarns have a dTex of from 40 to 340, more preferably from 40 to 180.

The upper surface layer is preferably such that liquids and air can easily pass there through and into the spacer layer and the spacer fabric is preferably such that it has an ability to conduct liquid away from the surface and dissipate it through the fabric structure, and such that it permits passage of air through the structure.

The upper surface layer is preferably a warp knitted mesh, having generally oval-shaped holes as hereinbefore described of a size such that liquids can pass therethrough. The mesh size of the upper surface layer is preferably as large as possible to allow for drainage and ventilation purposes, but should not be so large as to cause discomfort when placed next to the skin. The oval-shaped holes preferably have a length of from 3.5 to 4.5 mm and a width of from 2 to 3 mm. A mesh having an average hole area of from 7 to 9 mm², preferably around 8 mm² has been found to give particularly good results.

The average width of the individual sinusoidal mesh strands in the upper surface layer is from 0.1 to 4 mm, preferably from 0.5 to 3mm, such as, for example, about 1 to 2 mm. Each mesh strand preferably comprises from 4 to 6 fibres in the strand. The sinusoidal mesh strands preferably have a periodicity (distance between successive peaks or troughs) of from 4 to 8mm, preferably from 5 to 7mm, for example, about 6mm.

Preferably the ratio of the average area of a hole of the mesh to the average width of a mesh strand in the upper surface layer is from 9:1 to 7:2, for example, 5:1.

The oval-shaped holes are formed by one or more threads joining adjacent sinusoidal mesh strands together. Preferably the parallel sinusoidal strands are offset from one another lengthwise, such that a peak of one strand faces a trough of an adjacent strand. The peaks and troughs of adjacent strands are preferably spaced apart by a distance of at least 0.25mm, more preferably from 0.4 to 1.2mm and most preferably from 0.5 to 1.0mm.

The threads are preferably parallel, and preferably of length from 0.4 to 1.2mm, most preferably 0.5 to 1.0mm. Preferably the threads have a dTex of from 40 to 180.

Preferably the upper surface layer of the spacer fabric is such that liquids of viscosity of at least 20 x 10⁻³ N/m (20 dynes per centimetre) and more preferably of at least 30 x 10⁻³ N/m (30 dynes per centimetre) can pass through the upper surface and into the spacer layer without lying on the surface.

Preferably the upper surface of the spacer fabric has a grade of less than 1 when tested in accordance with the Oil Repellency Rating AATCC test method 118-1989.

The breathability of the upper surface layer is preferably such that, when placed face down on the fabric, a baby can continue to breath relatively normally.

A suitable air permeability test providing a measure of the breathability of a fabric, i.e. the ease with which air passes through the fabric structure, is BS 4578:1970 (1991) Measurement of Restriction of Airflow. Preferably the spacer fabric has a value of less than 5 mm H2O, more preferably less than 2.0mm H₂O, most preferably less than 1mm H₂O, when tested in accordance with BS 4578:1970 (1991).

Preferably the upper surface layer comprises a warp knitted mesh of multifilament yarns.

Preferably there are incorporated in the upper surface layer inherently wicking fibres or a wicking fibre construction as described and claimed in UK Patent No. 2352735B.

In this specification the term "wicking fibre" is intended to mean a fibre which, by virtue of its shape and configuration, and/or filament dTex, has inherent wicking properties, whereby liquid can be transported along the fibre by capillary action. Similarly the term "wicking construction" is intended to mean a fibre construction, comprising two or more fibres, which construction has inherent wicking properties, whereby liquid can be transported along the fibre construction by capillary action.

Preferred wicking fibres for use in the upper surface layer are multifilament synthetic fibre yarns sold for their inherent wickability. Such fibres have enhanced capillary action by virtue of their shape and configuration. The enhanced wicking properties of so-called wicking fibres can be achieved, for example, by various different fibre cross-sectional structures, preferably providing at least one longitudinal channel which permits faster liquid transport by capillary action. All wicking fibres have a capability of wicking at a significantly greater rate and to a greater distance than conventional multifilament fibres of similar dTex. They can, for example, have a complex cross-section which provides a plurality of longitudinal channels to conduct liquid along the fibre at a rate and distance greater than a comparable conventional multifilament fibre with a circular cross-section. Fabrics knitted from inherently wicking fibres can have a drying rate of up to 20%, more preferably 30% and most preferably 50% faster than cotton, and up to 5%, and more preferably 10%, faster than conventional synthetic fibres. Preferably a fabric made from an inherently wicking fibre has a moisture loss of at least 5%, more preferably at least 10%, greater than a fabric made from a conventional synthetic fibre having a circular cross-section after 30 minutes.

Suitable synthetic fibre yarns include polyesters and polyamides, although polyesters are preferred, due to their greater heat stability. Preferred multi-filament yarns have a dTex of from 40 to 340, more preferably from 40 to 180. An example of a suitable wicking fibre is CoolMax™, which is a four channel Dacron™ polyester fibre with a special cross-sectional structure comprising three intersecting circles manufactured by Du Pont. Another potentially suitable wicking fibre is CoolMax Alta™, also manufactured by Du Pont.

Wicking fibre constructions that can be used in the upper surface layer usually comprise two or more synthetic fibres of different dTex, knitted in layers. A typical wicking fibre construction comprises an upper layer of a relatively coarse fibre and a lower layer of a relatively fine fibre or microfilament.

Suitable synthetic fibres for the wicking fibre construction include polyesters and polyamides, although polyesters are preferred due to their greater heat stability. The wicking fibre construction can, for example, comprises an upper layer of a coarse multifilament yarn having a filament dTex of from 6 to 3, and a lower layer of a microfilament yarn having a dTex of from 1.1 to 0.3.

In addition to its inherent wicking properties, the upper surface layer can also aid liquid transport by allowing liquids to pass through itself into the spacer layer.

In certain embodiments of the invention, at least the upper surface layer of the spacer fabric can also comprise an anti-bacterial yarn which is preferably of the type that also retards the growth of mould, mildew and fungus. Incorporation of an inlay of the anti-bacterial yarn can provide a safer and more hygienic spacer fabric. Other inlays which can be used include, for example, thermoregulating fibres.

The linking threads of the spacer layer preferably comprise a mono-filament yarn which traverses back and forth between the upper and lower surfaces. By omitting multi-filament linker threads from the spacer layer, the air volume of the spacer layer can be increased, providing improved air permeability and heat dissipation. In a preferred spacer fabric of the invention, the number of mono-filament linker threads in the spacer layer is preferably from 100 to 400 threads per square centimetre, for example about 286 threads per square centimetre.

Whilst the mono-filament linking threads in the spacer layer can be individually spaced apart and perpendicularly arranged with respect to the upper and lower surface layers, they are preferably arranged such that each pair, or group, of threads is in the form of a V-shape, when the fabric is viewed in cross-section, with the angle of the V preferably being from 5° to 55°, for example about 27° to about 32°. The V-shaped pairs or groups of threads can form a zig-zag pattern, and each individual thread can have a horizontal midsection which is inlaid into the upper surface layer.

Preferably at least 50% and more preferably 100% of the linking threads are arranged in V-shaped formations.

By arranging for pairs or groups of threads linking the upper and lower surfaces to lie at opposed angles to the perpendicular distance between the upper and lower surfaces, it is possible to improve the resistance of the spacer fabric to "flopping over" when subjected to a compressive force. This "flopping over" is highly undesirable since it can result in the complete flattening of the spacer fabric and a loss of the spacer layer with its properties of breathability and heat dissipation. As the linking threads are angled in alternate directions the spacer fabric can achieve a comfortable resilient feel whilst still retaining breathability, heat dissipation and a resistance to crushing.

The linking threads preferably have a sufficient stiffness to resist complete crushing of the fabric by the distributed weight of a baby, and yet have sufficient resilience to impart springiness or "give" to the fabric for comfort. Preferred mono-filament yarns for use as linking threads have a dTex of from 22 to 115, and can be made, for example, from a polyamide such as Nylon, a polypropylene, or most preferably, a polyester.

Preferably the spacer fabric of the invention is such that the spacer layer requires a work of compression, as measured by BS 4098:1975 of at least 50 J/metre², preferably at least 60 J/metre², with a maximum of around 350J/m² and a thickness recovery of at least 50%, preferably at least 75%, and a compression recovery of at least 65%, preferably at least 75%.

Preferably the spacer fabric of the invention is such that in the spacer layer the ratio of the volume of free space to the volume of linker threads is greater than 40, preferably greater than 100.

In preferred embodiments of the invention, the upper surface layer has a construction wherein the mono-filament linker threads of the spacer layer are effectively surrounded by softer multi-filament yarns in order to give a still softer surface feel. This construction can be achieved, for example, using a Liba-DPL machine, and a combination of closed and open stitches relative to the different yarns and threads. Preferably an open stitch is applied to the surface multi-filament yarns, and a closed stitch to the mono-filament linker threads.

Surrounding the mono-filament linker threads with multi-filament yarns in the upper surface layer spreads the point of load of each mono-filament linker thread over a larger area and imparts greater resilience and improved compression anti-fatigue characteristics to the fabric.

In preferred spacer fabrics according to the invention the surface mesh is fully supported by the mono-filament linker threads.

The dimensionally stable lower surface layer of the spacer fabric of the invention is preferably knitted with stitches having a plurality of loops, which can be achieved, for example, by using two guide bars instead of one, and using a Liba-DPLM machine. The number of stitches is reflected in the gauge of the knitting machine used, and preferably the machine has a gauge of at least 16 and preferably 16, 22, 24, or 28. By "dimensionally stable" is meant that the lower surface layer retains its integrity even after washing and crumpling.

In certain embodiments of the invention, the lower surface of the spacer fabric is provided with a liquid impermeable layer which can be obtained, for example, by direct coating of the lower surface of the fabric with a liquid-impermeable polymeric material, by impregnation of a liquid-impermeable polymeric material, or by transfer coating, or laminating a film of liquid-impermeable polymeric material thereto, to provide a tightly adherent, liquid-impermeable, backing layer or impregnated layer.

Preferably the liquid-impermeable layer is provided by laminating a flexible backing layer of a suitable polymeric material, for example, a polyurethane film, to the lower surface of the fabric by means of an adhesive. The layer of polymeric material is preferably from 10 to 30 microns in thickness, and good results and good flexibility have been achieved using a 25 micron thick polyurethane layer. Other polymeric film materials, such as, for example, polyethylene and polyvinylchloride may also be used in appropriate circumstances.

Where an adhesive is used for laminating, this may be solvent or heat activated, or cold-cured but the amount of heat and pressure used in the lamination process must neither be sufficient to compress the resultant laminate unduly, nor to cause permanent damage thereto. Preferably the adhesive, when set, forms a flexible film in order to prevent crumpling and flexing of the material without cracking of the film.

Preferably the backing layer achieves a pass as waterproof when tested in accordance with BS EN 20811:1992.

The backing layer is preferably such that it can be repeatedly machine washed and dried in a tumble dryer without undue shrinkage or permanent damage thereto.

The lower surface layer of the spacer fabric is preferably a multi-filament or spun-filament warp knitted fabric, and, for example, there may be used a multi-filament yarn having a dTex of from 40 to 230, for example, about 78 dTEX. Polyamide or polyester yarns are examples of suitable multifilament yarns which can be used, although polyester yarns are preferred.

The spacer fabric as a whole should of course have a high wickability, which is defined as the ability of the fabric to conduct liquid away from the area of initial contact and form a relatively thin liquid film within the fabric structure. Wickability of the fabric as a whole can be measured in accordance with TTM 1428:92 (FDC.348) by suspending test specimens from spring clips vertically over a beaker of distilled water and measuring the height to which the liquid rises in a given time. Preferably the spacer fabric is such that the wicked liquid rises to a height of at least 50mm, preferably at least 100mm, when tested in both the warp and weft directions, in a time of 30 minutes. Prior to testing the specimens are conditioned for a minimum of 16 hours in a standard atmosphere of 20°C/65% Relative Humidity ±2.

A further measure of the ability of the spacer fabric to conduct liquid away from its surface and dissipate it through the fabric structure is a water dispersion test in which a solution containing a suitable dye is used to measure the spread of liquid into and through the fabric. In this test, a measured amount of liquid (0.5ml) is applied to the fabric upper surface. The dimensions of the area stained due to the spread of liquid are measured over time. In a preferred spacer fabric in accordance with the invention the dimensions of the spread of water containing dye are at least 5.5cm by 2.5cm and the spread of liquid reaches near equilibrium in about 15 minutes.

The fabric preferably has good heat dissipation, such that it can dissipate heat rapidly away from a hot body. Preferably the fabric is such that the temperature of the fabric when placed under a hot plate with an initial temperature of 34°C does not exceed 25°C and more preferably 22°C after 10 minutes.

In certain preferred constructions according to the invention, where the liquid impermeable layer is not laminated to the spacer fabric, it is found that the spacer fabric makes less noise when its surface is rubbed softly, thereby improving the comfort of a cot mattress produced therefrom by reducing rustling.

In one embodiment according to the present invention, a cot mattress can be formed by providing a mattress core, a mattress cover comprising a spacer fabric according to the invention, and a liquid impermeable layer therebetween. For example, a mattress core, which can be either a foam plastics core or a sprung interior mattress core, can be provided with a liquid impermeable waterproof underlay, and the spacer fabric of the invention can be formed into a removable mattress cover therefor. An advantage of this construction is that the spacer fabric without the waterproof laminated layer is likely to be more resistant to creasing and distortion when washed at high temperatures. In this embodiment the mattress core is preferably completely enclosed with a waterproof film layer in .order to prevent liquids from reaching the core. Complete enclosure of a foam mattress core, for example, by the use of a water proof plastics underlay, is important, since if the mattress becomes wet it can form depressions which do not recover when dry.

The resistance of a laminated mattress cover according to a further aspect of the invention, wherein the cover comprises the spacer fabric and a waterproof plastics backing layer, to distortion and creasing during a 60°c wash, may be improved by cross-linking the plastics layer, either before or after the lamination step. Cross-linking can be carried out by, for example, electron beam irradiation, chemical cross-linking, or other techniques known to the art. In this aspect of the invention, cross-linking of the waterproof backing can be applied to laminated mattress covers according to the present invention, and also to the backing layer of laminated spacer materials produced in accordance with GB2305191B.

The foam plastics core or body of a foam mattress according to the invention preferably comprises an open cell polymeric foam material, for example, foamed polyurethane, and very good results have been obtained using Vitafoam (RTM), a polyurethane foam comprising Melamine as a fire retardant additive. Preferably the foam plastics core or body is permeable to air, although with certain spacer materials of high breatheability this may not be essential. Perforation of the foam plastics core is not usually required.

Where the spacer fabric is used as a mattress cover or mattress protector, it is preferably removable from the mattress core or body for washing purposes and, for example, the cover material or mattress protector may be a loose cover, or provided with a zip at one or more edge regions to permit such removal.

In order to reduce the manufacturing cost of the cot mattress, it is possible to provide the spacer fabric as the top surface layer only of the mattress, the sides and lower surfaces being made of cheaper standard mattress cover fabric material.

In preferred embodiments of the invention, the mattress achieves a pass under BS Standard 7177 for Resistance to Ignition of Mattresses, Divans and Bed Bases, and BS Standard 1877 Fire Retardancy Test for Mattresses and Bumpers for Childrens' Cots, Perambulators and Similar Domestic Articles and is devoid of fire retardant additives comprising antimony, phosphorus or arsenic.

Spacer fabrics can be knitted, for example, on Raschelmachines with two needle bars. Depending upon the nature of the spacer fabric and its physical requirements, a minimum of four guide bars, and normally four to six or more guide bars, are used. In addition to the requirements set out hereto, the thickness of the yarn used for the spacer threads is influenced by the distance between the upper and lower surfaces, the desired softness of the upper surface and whether the central layer is knitted with one guide bar or with two guide bars knitting in opposition to each other. The manufacturing methods for spacer fabrics are discussed in the brochure "Spacer Fabrics - Manufacturing Methods and Applications" published in 1994 by Karl Mayer Textilmaschinenfabrik GmbH. In the spacer fabrics of the present invention, the distance between the upper and lower surfaces, that is, the width of the spacer layer, is preferably from 2 to 6mm, more preferably about 3mm.

Preferred embodiments of a spacer fabric and a cot mattress and mattress cover according to the invention are described in the following Examples:

### EXAMPLE 1

A spacer fabric not necessarily in accordance with the invention but which may aid in its comprehension is knitted on a RD6N machine using two needle bars and six guide bars. The sequence of operation is as follows:

| | |
|---|---|
| GUIDE BAR 1 | 6-6-3-3/0-0-3-3/6-6-3-3/0-0-3-3/6-6-4-4/13-3-6-6/9-9-6-6/3-3-5-5// |
| GUIDE BAR 2 | 3-3-6-6/9-9-6-6/3-3-6-6/9-9-6-6/3-3-4-4/6-6-3-3/0-0-3-3/6-6-3-3/0-0-3-3/6-6-4-4// |
| GUIDE BAR 3 | 1-0-0-0/0-1-1-1// |
| GUIDE BAR 4 | 1-0-2-3/1-0-2-3// |
| GUIDE BAR 5 | 2-3-1-0/2-3-1-0// |
| GUIDE BAR 6 | 0-0-0-2/2-2-2-0// |

| | |
|---|---|
| Guide bars 1 and 2 form the top mesh surface. | |

Guide bars 4 and 5 could have different movements for the linking threads, which could in an alternative manufacturing method use only one instead of two guide bars. It would also be possible to use two half set guide bars in opposition instead of one.

Guide bars 5 and 6 could again have different movements for the production of different fabric backing types.

The construction notation is given in steps of 2 i.e. 0-1-2-3-4, where each number represents a movement (or non-movement of the guide bar over one needle space).

Eg. 0-1 is a movement over one needle. 0-2 is a movement over two needles.

The numbers between the / marks represent the movement with respect to a needle bar or bars.

Eg. 1-0-1-2// will mean the guide bar knitting over both needle bars (to use the linking threads).

1-0-1-1// will mean the guide bar knitting only on one needle bed, as there is no movement (2-2) on the second needle bar.

In a preferred example (again, not necessarily within the invention, but which may aid in its comprehension), by way of example only, the yarn dTEX (thickness) is as follows:
Bars 1, 2 and 3 - 78 dTEX polyester
Bars 4 and 5 - 33 dTEX polyester
Bar 6 - 78 dTEX polyester

The resultant spacer fabric has a thickness of 3mm, an upper surface mesh hole average area of 8mm² and an average mesh strand width of 1.5mm.

The spacer fabric can be slit to 60cm wide and made up into a zip-off cover for a cot mattress. The foam core of the cot mattress is a 10cm thick polyurethane foam material of grade 35M.

All the polyester yarns used in the manufacture of the spacer fabric exemplified, and the polyurethane foam of the mattress core, are chosen to be substantially free of arsenic and antimony, and to contain less than 12 parts per million, preferably to be substantially free, of phosphorus.

Whilst there is no specific test for fabric "feel" or "handle", subjectively, a spacer fabric, mattress cover and mattress produced as described above have improved softness to the touch, and have a feel closely resembling comparable soft fabric materials. Samples of the spacer fabric, mattress cover and mattress produced as described above were subjected to the following tests, with results and conclusions as set out below. The comparison fabric is a fabric produced in accordance with GB2305191B, EP1204791B and GB2352735B.

### 1. Air Permeability Test

This is to assess the breathability of the fabric, i.e. the ease with which air passes through the fabric structure.

Test Method: BS 6595:1985 clause 3.3; BS 4578:1970 (1991) Measurement of Restriction of Airflow.

The closer the result is to zero the better the airflow through the mattress cover.

The results are as follows:

| | New fabric | Comparison |
|---|---|---|
| Upper fabric surface | 2.3 mm H₂0 | 1.4 mm H₂0 |

The results indicate that the spacer fabric cover of the present invention has a slightly lower permeability than the comparison, but still excellent breathability.

After washing in accordance with BS49236A at 40°C and line drying, the air flow restriction of the spacer material mattress cover of the invention is still very low (3.1 mm H₂O).

### 2. Liquid Dissipation Tests

These demonstrate the ability of the fabric to take liquid away from the surface and dissipate it through the fabric structure.

### 2(a) Liquid Flow Test

Liquid flow from the surface of the fabric into the structure of the fabric is measured according to AATCC test method 118-1989.

The closer the rating is to zero, the more liquids are taken into the fabric. The new fabric had an initial rating less than 1, which indicates that liquids of all tested viscosities soaked into the fabric structure and proves liquid would not sit on the fabric surface. After washing and dry cleaning the rating was still less than 1.

### 2(b). Wicking test (IHTM017 based on TTM1428:92 (FDC. 348)

Test specimens are suspended over a beaker of distilled water and the height to which the liquid rises is measured over time.

The new fabric and the comparison are tested in both fabric directions.

The results are as follows:

| Wicking Rate | Comparison | New Fabric |
|---|---|---|
| Warp direction 1 min | 39mm | 45mm |
| Warp direction 5 mins | 71mm | 78mm |
| Warp direction 30 mins | Exceeded clips @ 24 min | 128mm |
| Warp direction 1 hr | ---- | Exceeded clips @ 36 min |
| Weft direction 1 min | 38mm | 23mm |
| Weft direction 5 mins | 70mm | 44mm |
| Weft direction 30 mins | exceeds clips @ 29 mins | 76mm |
| Weft direction >1hr | ----- | Exceeded clips @ 88 min |

Whilst the results for the new fabric are slightly inferior to those of the comparison, they are still very good, especially in the warp direction, and it can be seen that the wicking rate of the new fabric in the warp direction actually exceeds that of the comparison initially.

### 3. Dimensional Stability to Washing

This test was carried out using wash cycle 2A, 60° C with tumble drying in accordance with BS EN 26330:1994.

| | New Fabric | Comparison |
|---|---|---|
| Dimensional change | length -2.0% | length -2.8% |
| | width -3.0% | width -2.7% |

The results show that both the new fabric and the comparison had minimal dimensional change after washing and tumble drying. The new fabric had less length-wise shrinkage but slightly more width-wise shrinkage.

### 4. Thickness Compression and Recovery Test

Five samples of the fabric of the invention are tested following the procedure described in BS4098:1975, and the results averaged.

| | New Fabric (averaged) | Comparison |
|---|---|---|
| Original thickness | 3.0mm | 4.1mm |
| Compression | 2.6mm | 3.2mm |
| Thickness recovery | 87.6% | 86.4% |
| Compression recovery | 82.9% | 82.7% |

The results show that the new fabric has a slightly improved thickness recovery and compression recovery after compression.

### 5. Wettability of Fabric

Wettability was tested in accordance with BS 4554:1970. Initially both the new fabric and the comparison were wetted in less than one second. After washing the new fabric wetted in from three to 27 seconds.

### 6. Fire Retardancy Test

A mattress made from a fabric in accordance with the invention is tested for fire retardancy to the standard laid down in the Furniture and Furnishing (Fire Safety) Regulations 1988. The result is a pass.

An embodiment of a spacer fabric according to the invention will now be described, by way of example only, with reference to the accompanying Drawings, in which:
Figure 1 shows a plan view of the upper face of the fabric; and
Figure 2 shows the fabric in sectional side elevation.

Referring to Figure 1, the spacer fabric illustrated generally at 1 has an upper face 2 comprising a warp knitted multifilament mesh having parallel sinusoidal strands 3 of width 2mm and periodicity (distance between successive peaks or troughs) of 6mm. The parallel sinusoidal strands are offset from each other such that a peak 4 of one strand is adjacent a trough 5 of an adjacent strand. Adjacent peaks 4 and troughs 5 of the strands are joined by four straight threads 6 of length 0.5 to 0.6mm, forming oval holes 7 of length 4mm and width 2.5mm. The strands 3 lie flat to the surface of the spacer fabric such that the fabric has a smooth, comfortable feel and are spaced apart to give a soft handle to the fabric.

In Figure 2 there is shown the spacer layer 8, having monofilament polyester spacer threads 9, disposed in generally V-shaped groups 10, with an acute angle a, as illustrated, between threads of opposed inclination. The lower surface 11 of the spacer fabric 1 is knitted from multifilament polyester threads to form a substantially dimensionally stable layer. Individual spacer linking threads such as 12, illustrated as a thicker line, have sections 13, 14, angled in opposed directions, and a horizontal midsection 15 which is inlaid in the upper surface layer 2.

The reader's attention is directed to all papers and documents which are filed concurrently with or previous to this specification in connection with this application and which are open to public inspection with this specification.

All of the features disclosed in this specification (including any accompanying claims, abstract and drawings), and/or all of the steps of any method or process so disclosed, may be combined in any combination, except combinations where at least some of such features and/or steps are mutually exclusive.

## Claims

1. A flexible spacer fabric (1), the fabric (1) having a liquid permeable and breathable upper surface layer (2), a heat and liquid dissipating spacer layer (8), and a dimensionally stable lower surface layer (11), wherein the upper surface layer (2) comprises a knitted mesh comprising sinusoidal mesh strands (3) extending in parallel across the upper face of the fabric (1), said strands being spaced apart and linked at adjacent points (5) by one or more straight threads (6) forming holes (7), bounded by the mesh strands (3) and threads, of generally oval shape, wherein the average width of the mesh strands (3) in the upper surface layer (2) is from 0.1 mm to 4 mm, and the parallel sinusoidal strands (3) are offset from one another lengthwise, such that a peak of one strand (3) faces a trough of an adjacent strand (3), **characterised in that** facing peaks and troughs are joined by four or more threads, to form the oval-shaped holes (7).

2. A fabric (1) according to Claim 1,
wherein the upper surface layer (2) comprises a warp knitted mesh of synthetic fibres; or
wherein the average length of a hole (7) in the mesh is from 3.5 to 4.5 mm and the average width of a hole (7) is from 2 to 3 mm; or
wherein the mesh average hole (7) area is from 7 to 9 mm²; or
wherein the average width of the sinusoidal mesh strands (3) in the upper surface layer (2) is from 0.5 to 3 mm; or
wherein the periodicity of the sinusoidal mesh strands (3) is from 4 to 8 mm.

3. A fabric (1) according to claim 1, wherein the peaks and troughs of adjacent strands (3) are spaced apart by a distance of from 0.4 to 1.2 mm.

4. A fabric (1) according to any one of claims 1 to 3, in which the threads are at least one of:
parallel; or
of length from 0.4 to 1.2 mm.

5. A fabric (1) according to any one of the preceding claims, wherein the ratio of the average hole area to the average width of the mesh strands (3) in the upper surface layer (2) is from 9:1 to 7:2.

6. A fabric (1) according to any one of the preceding claims, wherein the upper surface layer (2) is knitted from multifilament synthetic yarn.

7. A fabric (1) according to Claim 6, wherein the multifilament yarn has a dTEX of from 40 to 180.

8. A fabric (1) according to any one of the preceding claims,
wherein the upper surface layer (2) is such that liquids of viscosity of at least 30 x 10⁻³ N/m can pass through the upper surface (2) and into the spacer layer (8) without lying on the surface (2); or
wherein the upper surface (2) of the fabric (1) has a grade of less than 1 when tested in accordance with the Oil Repellency Rating AATTC test method 118-1989; or
which has a value of less than 2.0 mm H₂O of water, when tested in accordance with BS4578:1970.

9. A fabric (1) according to any one of the preceding claims, wherein the upper surface layer (2) comprising wicking fibres or a wicking fibre construction.

10. A fabric (1) according to Claim 9, wherein the wicking fibres comprise multifilament synthetic fibre yarns.

11. A fabric (1) according to Claim 9 or 10, wherein the multifilament wicking fibre yarns have a dTEX of from 40 to 180.

12. A fabric (1) according to Claim 9, wherein the wicking fibre construction comprises an upper layer of a coarse multifilament yarn having a filament dTEX of from 6 to 3 and a lower layer of a micro filament yarn having a dTEX of from 1.1 to 0.3.

13. A fabric (1) according to any one of the preceding claims, in which the linking threads of the spacer layer (8) consist solely of a monofilament yarn.

14. A fabric (1) according to claim 13, wherein the number of monofilament linking threads in the spacer layer (8) is from 100 to 400 threads per square cm.

15. A fabric (1) according to claim 13 or 14, wherein the monofilament threads are arranged such that each pair, or group, of threads is in the form of a V-shape.

16. A fabric (1) according to claim 15, wherein an angle of the V is from 5° to 55°.

17. A fabric (1) according to claim 15 or 16, wherein substantially a 100% of the linking threads are arranged in V-shaped formations.

18. A spacer fabric (1) according to any one of claims 13 to 17,
wherein individual monofilament linking threads have sections angled in opposed directions and a midsection which is inlaid in the upper surface layer (2); or
wherein the monofilament linking threads have a dTEX of from 22 to 115; or
wherein the monofilament linking threads comprise a polyester; or
wherein the upper surface layer (2) has a construction wherein the monofilament linking threads of the spacer layer (8) are surrounded by softer multifilament yarns; or
such that the spacer layer (8) requires a work of compression as measured by BS4098:1975 of at least 60 J/m²; or
which has a thickness recovery as measured by BS4098:1975 of at least 75%; or
which has a compression recovery as measured by BS4098:1975 of at least 75%; or
such that in the spacer layer (8) the ratio of the volume of free space to the volume of linking threads is greater than 100; or
wherein the dimensionally stable lower surface layer (11) is knitted with stitches having a plurality of loops.

19. A fabric (1) according to any one of the preceding claims, wherein the lower surface layer (11) comprises a multi-filament or spun-filament warp knitted fabric.

20. A fabric (1) according to claim 19, wherein there is used a multi filament yarn having a dTEX of from 40 to 230.

21. A fabric (1) according to claim 19 or 20, wherein the multi filament yarn comprises a polyester.

22. A mattress cover which comprises a flexible spacer fabric (1) according to any of claims 1 to 21 and a liquid impermeable lower surface layer (11).

23. A mattress cover according to claim 22, wherein the liquid impermeable lower surface layer (11) is laminated to the spacer fabric (1).

24. A cot mattress comprising a foam plastics core or a spring mattress core and a cover comprising an outer layer of flexible spacer fabric (1) according to any one of claims 1 to 21 and a liquid impermeable inner layer.

25. A cot mattress according to claim 24, wherein the mattress core comprises an open cell polymeric foam material.

## Patentansprüche

1. Flexibles Abstandshaltergewebe (1), wobei das Gewebe (1) eine flüssigkeitsdurchlässige und atmungsaktive obere Oberflächenschicht (2), eine wärme- und flüssigkeitsableitende Abstandshalterschicht (8) und eine formstabile untere Oberflächenschicht (11) aufweist, wobei die obere Oberflächenschicht (2) ein gestricktes Geflecht umfasst, das sinusförmige Flechtsträhnen (3) umfasst, die sich parallel über die obere Seite des Gewebes (1) erstrecken, wobei die Strähnen voneinander beabstandet und an benachbarten Punkten (5) durch ein oder mehr gerade Fäden (6), die Löcher (7) bilden, verbunden sind, begrenzt durch die Flechtsträhnen (3) und Fäden mit im Allgemeinen ovaler Form, wobei die durchschnittliche Breite der Flechtsträhnen (3) in der oberen Oberflächenschicht (2) 0,1 mm bis 4 mm beträgt, und
die parallelen sinusförmigen Strähnen (3) voneinander der Länge nach versetzt sind, so dass eine Spitze einer Strähne (3) einem Tal einer benachbarten Strähne (3) zugewandt ist, **dadurch gekennzeichnet, dass** zugewandte Spitzen und Täler durch vier oder mehr Fäden verbunden sind, um die ovalen Löcher (7) zu bilden.

2. Gewebe (1) nach Anspruch 1,
wobei die obere Oberflächenschicht (2) ein gestricktes Kettgeflecht aus synthetischen Fasern umfasst; oder
wobei die durchschnittliche Länge eines Lochs (7) im Geflecht 3,5 bis 4,5 mm beträgt und die durchschnittliche Breite eines Lochs (7) 2 bis 3 mm beträgt; oder
wobei die Fläche des Flechtdurchschnittslochs (7) 7 bis 9 mm² beträgt; oder
wobei die durchschnittliche Breite der sinusförmigen Flechtsträhnen (3) in der oberen Oberflächenschicht (2) 0,5 bis 3 mm beträgt; oder
wobei die Periodizität der sinusförmigen Flechtsträhnen (3) 4 bis 8 mm beträgt.

3. Gewebe (1) nach Anspruch 1, wobei die Spitzen und Täler von benachbarten Strähnen (3) mit einem Abstand von 0,4 bis 1,2 mm beabstandet sind.

4. Gewebe (1) nach einem der Ansprüche 1 bis 3, wobei die Fäden wenigstens eines von Folgenden sind:
parallel; oder
mit einer Länge von 0,4 bis 1,2 mm.

5. Gewebe (1) nach einem der vorhergehenden Ansprüche, wobei das Verhältnis der Durchschnittslochfläche zur Durchschnittsbreite der Flechtsträhnen (3) in der oberen Oberflächenschicht (2) 9:1 bis 7:2 beträgt.

6. Gewebe (1) nach einem der vorhergehenden Ansprüche, wobei die obere Oberflächenschicht (2) aus synthetischem Mehrfachfadengarn gestrickt ist.

7. Gewebe (1) nach Anspruch 6, wobei das Mehrfachfadengarn einen dTEX von 40 bis 180 aufweist.

8. Gewebe (1) nach einem der vorhergehenden Ansprüche,
wobei die obere Oberflächenschicht (2) so ist, dass Flüssigkeiten mit einer Viskosität von wenigstens 30 x 10⁻³ N/m durch die obere Oberfläche (2) und in die Abstandshalterschicht (8) gelangen können, ohne auf der Oberfläche (2) zu liegen; oder
wobei die obere Oberfläche (2) des Gewebes (1) einen Grad von weniger als 1 aufweist, wenn sie gemäß dem Ölabweisung messenden Testverfahren AATTC 118-1989 gemessen wird; oder
die einen Wert von weniger als 2,0 mm H₂O von Wasser aufweist, wenn sie gemäß BS4578:1970 gemessen wird.

9. Gewebe (1) nach einem der vorhergehenden Ansprüche, wobei die obere Oberflächenschicht (2) Schweiß transportierende Fasern oder eine Schweiß transportierende Faserstruktur umfasst.

10. Gewebe (1) nach Anspruch 9, wobei die Schweiß transportierenden Fasern synthetisches Mehrfachfadenfasergarn umfassen.

11. Gewebe (1) nach Anspruch 9 oder 10, wobei die Schweiß transportierenden Mehrfachfadenfasergarne einen dTEX von 40 bis 180 aufweisen.

12. Gewebe (1) nach Anspruch 9, wobei die Schweiß transportierende Faserstruktur eine obere Schicht aus einem groben Mehrfachfadengarn mit einem Filament-dTEX von 6 bis 3 und eine untere Schicht aus einem Mikrofilamentgarn mit einem dTEX von 1, 1 bis 0,3 umfasst.

13. Gewebe (1) nach einem der vorhergehenden Ansprüche, wobei die verbindenden Fäden der Abstandshalterschicht (8) lediglich aus einem Einzelfasergarn bestehen.

14. Gewebe (1) nach Anspruch 13, wobei die Anzahl von Einzelfaser verbindenden Fäden in der Abstandshalterschicht (8) 100 bis 400 Fäden pro Quadratzentimeter beträgt.

15. Gewebe (1) nach Anspruch 13 oder 14, wobei die Einzelfaserfäden so angeordnet sind, dass jedes Paar, oder jede Gruppe, von Fäden eine V-Form aufweist.

16. Gewebe (1) nach Anspruch 15, wobei ein Winkel des V 5° bis 55° beträgt.

17. Gewebe (1) nach Anspruch 15 oder 16, wobei im Wesentlichen 100% der verbindenden Fäden in V-förmigen Formationen angeordnet sind.

18. Abstandshaltergewebe (1) nach einem der Ansprüche 13 bis 17,
wobei individuelle Einzelfaser verbindende Fäden Abschnitte aufweisen, die in entgegengesetzte Richtungen gewinkelt sind, und einen mittleren Abschnitt, der in die obere Oberflächenschicht (2) eingelegt ist; oder
wobei die Einzelfaser verbindenden Fäden einen dTEX von 22 bis 115 aufweisen; oder
wobei die Einzelfaser verbindenden Fäden Polyester umfassen; oder
wobei die obere Oberflächenschicht (2) eine Struktur aufweist, wobei die Einzelfaser verbindenden Fäden der Abstandshalterschicht (8) von weicherem Mehrfachfadengarn umgeben sind; oder
so dass die Abstandshalterschicht (8) eine Verdichtungsarbeit, wie sie von BS4098:1975 gemessen wird, von wenigstens 60 J/m² erfordert; oder
das eine Stärke-Rückverformung, wie sie von BS4098:1975 gemessen wird, von wenigstens 75% aufweist; oder
das eine Kompressions-Rückverformung, wie sie von BS4098:1975 gemessen wird, von wenigstens 75% aufweist; oder
so dass in der Abstandshalterschicht (8) das Verhältnis des Volumens von freiem Raum zum Volumen von verbindenden Fäden größer als 100 ist; oder
wobei die formstabile untere Oberflächenschicht (11) mit Stichen gestrickt ist, die eine Mehrzahl von Schlaufen aufweisen.

19. Gewebe (1) nach einem der vorhergehenden Ansprüche, wobei die untere Oberflächenschicht (11) ein gestricktes Mehrfachfaden- oder Spinnfaden-Kettgewebe umfasst.

20. Gewebe (1) nach Anspruch 19, wobei ein Mehrfachfadengarn mit einem dTEX von 40 bis 230 verwendet wird.

21. Gewebe (1) nach Anspruch 19 oder 20, wobei das Mehrfachfadengarn Polyester umfasst.

22. Matratzenbezug, der ein flexibles Abstandshaltergewebe (1) nach einem der Ansprüche 1 bis 21 und eine flüssigkeitsundurchlässige untere Oberflächenschicht (11) umfasst.

23. Matratzenbezug nach Anspruch 22, wobei die flüssigkeitsundurchlässige untere Oberflächenschicht (11) auf das Abstandshaltergewebe (1) geschichtet ist.

24. Kinderbettmatratze, die einen Schaumstoffkern oder einen Sprungfedermatratzenkern und einen Bezug umfasst, der eine äußere Schicht aus flexiblem Abstandshaltergewebe (1) nach einem der Ansprüche 1 bis 21 und eine flüssigkeitsundurchlässige innere Schicht umfasst.

25. Kinderbettmatratze nach Anspruch 24, wobei der Matratzenkern ein offenzelliges Polymerschaummaterial umfasst.

## Revendications

1. Tissu intercalaire souple (1), le tissu (1) ayant une couche de surface supérieure (2) perméable aux liquides et à l'air, une couche intercalaire (8) dissipant la chaleur et les liquides, et une couche de surface inférieure (11) stable d'un point de vue dimensionnel, dans lequel la couche de surface supérieure (2) comprend une maille tricotée comprenant des brins de maille sinusoïdaux (3) s'étendant en parallèle sur l'ensemble de la surface supérieure du tissu (1), lesdits brins étant espacés et reliés au niveau de points adjacents (5) par un ou plusieurs fils droits (6) formant des trous (7), délimités par les brins de maille (3) et les fils, d'une forme générale ovale, la largeur moyenne des brins de maille (3) dans la couche de surface supérieure (2) étant de 0,1 mm à 4 mm, et les brins sinusoïdaux parallèles (3) étant décalés les uns des autres longitudinalement, de telle sorte qu'un pic d'un brin (3) fait face à un creux d'un brin adjacent (3), **caractérisé par le fait que** des pics et des creux en regard sont réunis par au moins quatre fils, pour former les trous (7) de forme ovale.

2. Tissu (1) selon la revendication 1,
dans lequel la couche de surface supérieure (2) comprend une maille tricotée en chaîne de fibres synthétiques ; ou
dans lequel la longueur moyenne d'un trou (7) dans la maille est de 3,5 à 4,5 mm et la largeur moyenne d'un trou (7) est de 2 à 3 mm ; ou
dans lequel la surface de trou (7) moyenne de maille est de 7 à 9 mm² ; ou
dans lequel la largeur moyenne des brins de maille sinusoïdaux (3) dans la couche de surface supérieure (2) est de 0,5 à 3 mm ; ou
dans lequel la périodicité des brins de maille sinusoïdaux (3) est de 4 à 8 mm.

3. Tissu (1) selon la revendication 1, dans lequel les pics et creux de brins adjacents (3) sont espacés d'une distance de 0,4 à 1,2 mm.

4. Tissu (1) selon l'une quelconque des revendications 1 à 3, dans lequel les fils sont au moins l'un parmi :
parallèles ; ou
de longueur de 0,4 à 1,2 mm.

5. Tissu (1) selon l'une quelconque des revendications précédentes, dans lequel le rapport de la surface de trou moyenne à la largeur moyenne des brins de maille (3) dans la couche de surface supérieure (2) est de 9:1 à 7:2.

6. Tissu (1) selon l'une quelconque des revendications précédentes, dans lequel la couche de surface supérieure (2) est tricotée à partir de fil synthétique multifilament.

7. Tissu (1) selon la revendication 6, dans lequel le fil multifilament a un dTEX de 40 à 180.

8. Tissu (1) selon l'une quelconque des revendications précédentes,
dans lequel la couche de surface supérieure (2) est tel que des liquides de viscosité d'au moins 30 x 10⁻³ N/m peuvent passer à travers la surface supérieure (2) et dans la couche intercalaire (8) sans s'étendre sur la surface (2) ; ou
dans lequel la surface supérieure (2) du tissu (1) a un calibre de moins de 1 lorsqu'elle est testée conformément à la méthode de test AATCC 118-1989 de Classification du Caractère Oléofuge ; ou
qui a une valeur de moins de 2,0 mm H₂O d'eau, lorsqu'il est testé conformément à BS4578:1970.

9. Tissu (1) selon l'une quelconque des revendications précédentes, dans lequel la couche de surface supérieure (2) comprend des fibres de mèche ou une structure de fibres de mèche.

10. Tissu (1) selon la revendication 9, dans lequel les fibres de mèche comprennent des fils de fibres synthétiques multifilaments.

11. Tissu (1) selon l'une des revendications 9 ou 10, dans lequel les fils de fibres de mèche multifilaments ont un dTEX de 40 à 180.

12. Tissu (1) selon la revendication 9, dans lequel la structure de fibres de mèche comprend une couche supérieure d'un fil multifilament grossier ayant un dTEX de filament de 6 à 3 et une couche inférieure de fil microfilament ayant un dTEX de 1,1 à 0,3.

13. Tissu (1) selon l'une quelconque des revendications précédentes, dans lequel les fils de liaison de la couche intercalaire (8) consistent uniquement en un fil monofilament.

14. Tissu (1) selon la revendication 13, dans lequel le nombre de fils de liaison monofilaments dans la couche intercalaire (8) est de 100 à 400 fils par cm carré.

15. Tissu (1) selon l'une des revendications 13 ou 14, dans lequel les fils monofilaments sont disposés de telle sorte que chaque paire, ou groupe, de fils est dans la forme d'un V.

16. Tissu (1) selon la revendication 15, dans lequel un angle du V est de 5° à 55°.

17. Tissu (1) selon l'une des revendications 15 ou 16, dans lequel sensiblement 100 % des fils de liaison sont disposés dans des formations en V.

18. Tissu intercalaire (1) selon l'une quelconque des revendications 13 à 17,
dans dequel des fils de liaison monofilaments individuels ont des sections coudées dans des directions opposées et une section médiane qui est incrustée dans la couche de surface supérieure (2) ; ou
dans lequel les fils de liaison monofilaments ont un dTEX de 22 à 115 ; ou
dans lequel les fils de liaison monofilaments comprennent un polyester ; ou
dans lequel la couche de surface supérieure (2) a une structure dans laquelle les fils de liaison monofilaments de la couche intercalaire (8) sont entourés par des fils multifilaments plus souples ; ou
tel que la couche intercalaire (8) nécessite un travail de compression tel que mesuré par BS4098:1975 d'au moins 60 J/m² ; ou
qui a une récupération d'épaisseur telle que mesurée par BS4098:1975 d'au moins 75 % ; ou
qui a une récupération après compression telle que mesurée par BS4098:1975 d'au moins 75 % ; ou
tel que, dans la couche intercalaire (8), le rapport du volume d'espace libre au volume de fils de liaison est supérieur à 100 ; ou
dans lequel la couche de surface inférieure (11) stable d'un point de vue dimensionnel est tricotée avec des points ayant une pluralité de boucles.

19. Tissu (1) selon l'une quelconque des revendications précédentes, dans lequel la couche de surface inférieure (11) comprend un tissu tricoté en chaîne multifilaments ou à filaments filés.

20. Tissu (1) selon la revendication 19, dans lequel est utilisé un fil multifilament ayant un dTEX de 40 à 230.

21. Tissu (1) selon l'une des revendications 19 ou 20, dans lequel le fil multifilament comprend un polyester.

22. Couvre-matelas qui comprend un tissu intercalaire souple (1) selon l'une quelconque des revendications 1 à 21 et une couche de surface inférieure (11) imperméable aux liquides.

23. Couvre-matelas selon la revendication 22, dans lequel la couche de surface inférieure (11) imperméable aux liquides est laminée sur le tissu intercalaire (1).

24. Matelas de lit comprenant une âme en matière plastique mousse ou une âme de matelas à ressorts et un recouvrement comprenant une couche externe de tissu intercalaire souple (1) selon l'une quelconque des revendications 1 à 21 et une couche interne imperméable aux liquides.

25. Matelas de lit selon la revendication 24, dans lequel l'âme de matelas comprend une matière en mousse polymère à cellules ouvertes.
